# EUROPEAN PATENT SPECIFICATION

(11) **EP 0 399 706 B1**
(45) Date of publication and mention of the grant of the patent: **01.09.1993**
(21) Application number: 90305117.5
(22) Date of filing: 11.05.1990
(51) Int. Cl.: D06M 15/643

(54) **Method of treating fibrous materials**
Verfahren zur Behandlung von Fasermaterialien
Procédé de traitement de matériaux fibreux

(30) Priority: 24.05.1989 GB 8911970
(43) Date of publication of application: 28.11.1990
(73) Proprietor: Dow Corning Limited, London WC2R 0HF (GB)
(72) Inventor: Cray, Stephen Edward, South Glamorgan Wales (GB); Renauld, Franck André Daniel, B-1900 Overijse (BE)
(74) Representative: Vandamme, Luc Johan Roger

(56) References cited:
- US-A- 4 757 121

## Description

This invention relates to a method of treating fibrous materials and more specifically to a method of treating textile materials.

With the expression fibrous materials is meant fibres of synthetic or naturally occurring materials, for example wool, cotton, polyester, carbon and blends of these. The invention relates to the treatment of the fibres as such as well as to the treatment of fabrics or textiles incorporating the fibres.

It is known to treat fibrous materials with compositions comprising amine-containing silicon compounds for imparting desirable properties, e.g. softness, water repellency, lubricity and crease resistance thereto. The GB-A-1 491 747 for example provides a composition for treatment of synthetic fibres which comprises 1 part of certain aminosilanes and 1 to 20 parts of certain epoxysiloxanes. The GB-A-1 296 136 provides a process for the treatment of synthetic organic textile fibres which includes the treatment with a composition comprising either a) a mixture of an aminosiloxane and a polyepoxide, b) a mixture of a liquid epoxysiloxane and a polyamine or c) a mixture of a liquid epoxysiloxane and an aminosiloxane. However, these materials tend to give a certain amount of yellowing of the treated fibres. In the US-A-4 757 121 it is proposed to overcome the yellowing problem when treating synthetic fibre made waddings by using a composition comprising 100 parts by weight of a combination of two organopolysiloxanes composed of from 5 to 95% by weight of an amino-substituted organopolysiloxane, and 95 to 5% by weight of a second amino-substituted organopolysiloxane, which is a reaction product of a liquid amino-substituted organopolysiloxane and a liquid organic epoxy compound, from 1 to 50 parts by weight of an epoxy-containing alkoxy silane and from 1 to 50 parts by weight of a mono- epoxy compound.

We have found that an improved treating composition can be made by restricting the amine-containing organosiloxane to those which are prereacted with a monoepoxide.

According to the invention there is provided a method of treating fibrous materials, which comprises the application to fibrous materials of a composition comprising as sole amine-containing organosilicon compound the reaction product of a organopolysiloxane having at least one unit of the general formula 03-aSiXₐ R-NH-2 R' and at least one unit having the general formula 04-bSi-X_{b} with one or more monoepoxides, wherein X de- notes a monovalent hydrocarbon having up to 8 carbon atoms, R denotes a divalent alkylene group, R'denotes a hydrogen atom or a group of the formula R-Z, wherein Z is NHX, NH₂, NHRNH₂ or NHRNHX, a has a value of 1 or 2 and b has a value of 2 or 3.

The organopolysiloxane used in the preparation of the reaction product may be any siloxane polymer having at least 1 unit of the general formula and at least one unit having the general formula . Preferably it is a substantially linear polydiorganosiloxane polymer, although small amounts of units 2 which cause branching of the siloxane are possible. Such units, which should not be present in more than 5% of the total number of units, have the general structure O3SiX. The substituent X may be any hydrocarbon group having up to 8 carbon atoms, for example alkyl, aryl, alkenyl, alkylaryl and arylalkyl. Preferably X denotes a lower alkyl group. Preferably at least 80% and most preferably substantially all X groups are methyl groups. It is, however, possible that small amounts of other substituents are present on silicon atoms, for example hydroxyl or alkoxy groups. The group R is a divalent alkylene group, preferably having up to 8 carbon atoms, most preferably from 3 to 8 carbon atoms. Examples of the R group include dimethylene, propylene, isobutylene and hexylene. The groups R' may be hydrogen or a group of the formula RZ, wherein Z denotes a primary or secondary amine group or a diamine of the formula NHRNH₂ or NHRNHX. a has a value of 1 or 2, which means that the unit may be located in the siloxane chain or may be an end-unit of the siloxane chain. Examples of the amine-containing substituent are OSi(CH₃)(CH₂)₃NH₂, OSi(CH₃)CH₂CH(CH₃)CH₂NH₂, OSi(CH₃)CH₂CH(CH₃)CH₂NH(CH₂)₂NH₂, O_{½}Si(CH₃)₂CH₂CH(CH₃)CH₂NH(CH₂CH₃), O_{½}Si(CH₃)₂(CH₂)₃NH(CH₂)₃NH(CH₂)₃NH₂. The other units of the organopolysiloxane are units of the general formula wherein b has a value of 2 or 3 and X has the meaning as above. This means that the units may be present in the siloxane chain or as endgroups of the chain. It is preferred that polydiorganosiloxane having from to 10 to 1000 siloxane units, particularly from 100 to 500 units, most preferably about 400 units are used. The viscosity of the polydiorganosiloxane tends to determine the softness which is imparted to the treated materials, the higher the viscosity, the softer the finish. However, for reasons of practicality it is preferred to use those materials which are liquid at room temperature. It is also preferred that from 0.1 to 20 mole% of all siloxane units are units of the formula 03-aSiXₐ₋R-NH- R', preferably from 1 to 10%, most preferably from 1 to 4%. A particularly advantageous amount is 2%. Amounts above 10% are unlikely to contribute additional beneficial effects to the treated materials. Suitable organopolysiloxanes for the preparation of the reaction product for use in the method of the invention are known in the art and many are commercially available. They can be made by methods known in the art, for example by the condensation of aminofunctional silanes or hydrolysis products thereof with cyclic siloxanes in the presence of endblocking units, for example those provided by hexamethyldisiloxanes.

Monoepoxides employed in the preparation of the reaction product are organic compounds having one epoxy group. By the term epoxy is meant a group composed of oxirane oxygen attached to two vicinal carbon atoms. Monoepoxides which are suitable for use in the present invention are those wherein the substituent of the said vicinal carbon atoms are hydrogen, hydrocarbon groups or ether or ester containing hydrocarbon groups. Preferably one of the carbon atoms has only hydrogen atoms while the other carbon atom has an alkyl group attached to it, which may range from methyl to a linear C₂₁ alkyl group. Most preferred are those monoepoxides wherein the alkyl group has from 1 to 10 carbon atoms, especially from 1 to 4 carbon atoms. Examples of suitable monoepoxides are ethylene oxide, propylene oxide, butadiene monoxide, 2,3-epoxy-cyclopentane, substituted olefin oxides, e.g. 2, 3-epoxy-propylbenzene, epoxy alcohols, e.g. glycidol, 2,3-epoxy- cyclopentanol, 3,4-epoxy-6-methylcyclohexylmethane, glycidyl ethers, e.g. phenyl glycidyl ether, butyl glycidyl ether or glycidyl esters, e.g.glycidyl acetate. Preferred are those monoepoxides of the general formula wherein n has a value of from 0 to 20, preferably 0 to 8, most preferably 0 to 3.

The reaction product for use in the method of the invention may be prepared according to known methods. For example, the two reagents may be reacted together in the presence of a low molecular weight aliphatic alcohol or in the presence of a catalytic amount of water. The reaction can be carried out at room temperature in the presence of such catalyst but is preferably carried out at increased temperatures, for example temperatures of 50°C or more. In order to make the reaction more easily handled it may be carried out in the presence of a solvent, which may be the alcohol mentioned above or other suitable solvents. The amount of monoepoxide used in the reaction should be such that no more than 10% of all amine groups in the organopolysiloxane are retained unreacted in the reaction product. Where a primary amine group was present in the organopolysiloxane two monoepoxide molecules can react with the amine. It is preferred that the majority of the amino groups in the reaction product are tertiary amine groups, although the presence of secondary amine groups to the exclusion of tertiary amine groups is also acceptable. The amine groups in the reaction product may thus be tertiary, secondary, a mixture of these, or a mixture of either or both with up to a maximum of 10% primary amine groups.

It is important that the reaction product is used in the method of the invention, and not a mere mixture of the polydiorganosiloxane and the monoepoxide. Mere mixtures which contain polydiorganosiloxanes having relatively high amounts of primary amine groups are not satisfactory, since they will still display a yellowing of the treated materials. Even a mixture of the two components in the presence of water, e.g. by using an emulsion, is unsatisfactory as the yellowing upon treatment with such mixtures or emulsions is worse than treatment according to the invention. Preferably no primary amines are retained in the reaction product. Most preferably no secondary amines are present either in the reaction product.

The method of the invention comprises the application to fibrous materials of a composition comprising as sole amine-containing compound the reaction product as described above. This application may be done in any convenient way. Application methods which are suitable include padding, dipping and spraying of a composition comprising the reaction product. The compositions used may be in any suitable form, e.g. solutions, dispersions or emulsions. The dispersions may be in aqueous or solvent based materials while the emulsions are preferably oil-in-water type emulsions. Especially preferred are emulsions, particularly microemulsions according to European patent specification 138192. Compositions which are useful in the method of the invention may comprise other ingredients which are useful in treatment compositions forfibrous materials, e.g. fatty acid softeners. Other ingredients e.g. surfactants in the emulsions are also useful. It is, however, preferred that the composition comprises no amine-containing compounds other than the reaction product.

The method of the invention is suitable for the treatment of both naturally occurring and synthetic fibres, for example carbon fibres, polyester fibres, cotton fibres and blends of cotton and polyester fibres. The application may be done at the stage of making the fibres, at the stage of producing the fabrics or in a special treating step later, for example during laundering of a textile fabric. Application may be followed by drying at room temperature or at increased temperatures. After the drying stage a further heat treatment of the fibrous materials is preferred. The latter is particularly useful when the textile fabrics are treated at the time of their production. The presence of small amounts of primary amine groups on the reaction product will increase the durability of the finish on the fibrous materials, especially when they are subjected to laundering operations. Fibrous materials and textiles which are treated according to the method of the invention have an improved softener and lubricity, a pleasant feel and handle, without suffering from yellowing due to the treatment.

In a further aspect of the invention there is provided a fibrous material treated according to the method of the invention. Also included are fabrics or textiles incorporating fibres when treated according to the method of the invention.

There now follow a number of examples illustrating the invention in which all parts are expressed by weight unless otherwise mentioned.

### Examples 1 - 5

1 molar part of a polydiorganosiloxane compound of the average formula wherein R denotes -CH₂CH(CH₃)CH₂NHCH₂CH₃, was reacted with 2 molar parts of a monoepoxide having the average formula wherein n was 0, 1, 3, 7 and 9 respectively for Examples 1, 2, 3, 4 and 5 in the presence a mixture of 95 parts of methanol, 3 parts of isopropanol and 2 parts of water at a temperature of 50°C. This yielded a reaction product which is believed to have the average formula wherein R' denotes A bath was prepared with a 2.77% solution in perchloro ethylene of the reaction product prepared in Examples 1 to 5 in which a piece of polyester cotton (65/35) was treated by padding. The piece was heated to 110°C for 1 minute, followed by 2 minutes at 180°C after treatment. The piece had picked up 0.5% by weight of the reaction product.

### Example 6 - 10

1 molar part of a polydiorganosiloxane compound of the average formula wherein R denotes -CH₂CH(CH₃)CH₂NHCH₂CH₂NH₂, was reacted with 6 molar parts of a monoepoxide having the average formula wherein n was 0, 1, 3, 7 and 9 respectively for Examples 6, 7, 8, 9 and 10 in the presence a mixture of 95 parts of methanol, 3 parts of isopropanol and 2 parts of water at a temperature of 50°C. This yielded a reaction product which is believed to have the average formula wherein R' denotes A bath was prepared with a 2.77% solution in perchloro ethylene of the reaction product prepared in Examples 6 to 10, in which a piece of polyester cotton (65/35) was treated by padding. The piece was heated to 110°C for 1 minute, followed by 2 minutes at 180°C after treatment. The piece had picked up 0.5% by weight of the reaction product.

### Examples 11 - 15

1 molar part of a polydiorganosiloxane compound of the average formula wherein R denotes -CH₂CH(CH₃)CH₂NHCH₂CH₂NH₂, was reacted with 24 molar parts of a monoepoxide having the average formula wherein n was 0, 1, 3, 7 and 9 respectively for Examples 11, 12, 13, 14 and 15 in the presence of a mixture of 95 parts of methanol, 3 parts of isopropanol and 2 parts of water at a temperature of 50°C. This yielded a reaction product which is believed to have the average formula wherein R' denotes A bath was prepared with a 2.77% solution in perchloro ethylene of the reaction product prepared in Examples 11 to 15, in which a piece of polyester cotton (65/35) was treated by padding. The piece was heated to 110°C for 1 minute, followed by 2 minutes at 180°C after treatment. The piece had picked up 0.5% by weight of the reaction product.

### Examples 16 - 20

1 molar part of a polydiorganosiloxane compound of the average formula wherein R denotes -(CH₂)₃NHCH₂CH₂NH₂, was reacted with 24 molar parts of a monoepoxide having the average formula wherein n was 0, 1, 3, 7 and 9 respectively for Examples 16, 17, 18, 19 and 20 in the presence of a mixture of 95 parts of methanol, 3 parts of isopropanol and 2 parts of water at a temperature of 50°C. This yielded a reaction product which is believed to have the average formula wherein R' denotes A bath was prepared with a 2.77% solution in perchloro ethylene of the reaction product prepared in Examples 16 to 20, in which a piece of polyester cotton (65/35) was treated by padding. The piece was heated to 110°C for 1 minute, followed by heating at 180°C for minutes aftertreatment. The piece had picked up 0.5% byweight of the reaction product.

### Examples 21 - 22

1 molar part of a polydiorganosiloxane compound of the average formula wherein R denotes -(CH₂CH(CH₃)CH₂)NHCH₂CH₂NH₂, was reacted with 24 molar parts of a monoepoxide having the formula in the presence of a mixture of 95 parts of methanol, 3 parts of isopropanol and 2 parts of water at a temperature of 50°C. This yielded a reaction product which is believed to have the average formula wherein R' denotes A bath was prepared with a microemulsion, containing 1.4% of the reaction product prepared in Example 21, in which a piece of polyester cotton (65/35) was treated by padding. The piece was heated to 110°C for 90 seconds, followed by heating at 180°C for 2 minutes and 150°C for 5 minutes respectively for Examples 21 and 22 after treatment. The pieces had picked up 1 % and 0.5% by weight of the reaction product respectively.

### Example 23

1 mole of (CH₃0)₂Si(CH₃)CH₂CH(CH₃)CH₂NH(CH₂)₂NH₂ and methanol were added to a reaction vessel. 1.1 mole of 1,2 butyleneoxide were added through a dropping funnel and the mixture was heated under a nitrogen blanket to 50°C which was maintained for 1 hour. The product was stripped under reduced pressure on a rotary evaporator. 1 mole of the product was mixed with 3 moles of water and heated to 110°C to allow condensation of the silanes. After purification hexamethyldisiloxane and cyclic dimethylsiloxane were added to- getherwith an alkaline catalyst. The mixture was heated for 5 hours to 140°C and then neutralised. The filtered reaction prdouct had the formula wherein R' denotes The reaction product was applied to a piece of polyester cotton according to the method described for Example 22.

### Comparative Examples 1 - 10

A bath was prepared with a 2.77% solution in perchloro ethylene of the amino containing polydiorganosiloxane used in Examples 11 to 15 on its own, in which a piece of polyester cotton (65/35) was treated by padding. The piece picked up 0.5% by weight of the siloxane. (Comparative Example 1).

As in Comparative Example 1, but using a mixture of 1 molar part of the polydiorganosiloxane of Comparative Example 1 with 2 molar parts of propylene oxide, but not reacted. (Comparative Example 2).

Comparative Example 3 was a piece of untreated polyester cotton (blank) as used in Examples 11 to 15.

A bath was prepared with a 2.77% solution in perchloro ethylene of the amino containing polydiorganosiloxane used in Examples 16 to 20 on its own, in which a piece of polyester cotton (65/35) was treated by padding. The piece picked up 0.5% by weight of the siloxane. (Comparative Example 4).

Comparative Example 5 was a piece of untreated polyester cotton (blank) as used in Examples 16 to 20.

Comparative Example 6 was a microemulsion of a mixture of the two reactants of Example 21, in the same proportions and with the same concentration, in which a piece of polyester cotton (65/35) was treated by padding. The piece picked up 1% by weight of the siloxane.

Comparative Example 7 was a microemulsion of the amino containing polydiorganosiloxane of Example 21 on its own in the same concentration, in which a piece of polyester cotton (65/35) was treated by padding. The piece picked up 1% by weight of the siloxane.

Comparative Example 8 was a piece of untreated polyester cotton (blank) as used in Example 21.

Comparative Example 9 was a piece of untreated polyester cotton (blank) as used in Examples 22 and 23.

Comparative Example 10 was a microemulsion of the amino containing polydiorganosiloxane of Example 22 on its own in the same concentration, in which a piece of polyester cotton (65/35) was treated by padding. The piece picked up 0.5% by weight of the siloxane.

All comparative treated pieces of polyester-cotton were heated to 110°C for 1 minute followed by 2 minutes at 180°C for Comparative Examples 1 to 8 and 5 minutes at 150°C for Comparative Examples 9 and 10. The treated pieces of polyester cotton of Examples 1 to 23 were compared for softness and yellowing effect. It was found that the increase in molecular weight of the siloxane polymer used gave also an increase in the softness of the treated material. Within each series of similar molecules the best softness was obtained by those materials where n had a value of 0, 1 or 3.

The whiteness index of Examples 16 to 20 were measured using a Hunterlab Optical sensor, Model D25M and were compared with Comparative Examples 4 and 5. The following results were obtained.

The whiteness index of Example 11 was measured using a Hunterlab Optical sensor, Model D25M and compared with Comparative Examples 1, 2 and 3. The following results were obtained:

The whiteness index of Example 21 was measured using a Hunterlab Optical sensor, Model D25M and compared with Comparative Examples 6, 7 and 8. The following results were obtained:

The whiteness index of Examples 22 and 23 was measured using a Hunterlab Optical sensor, Model D25M and compared with Comparative Examples 9 and 10. The following results were obtained:

It can be seen from the results that the method according to the invention yields treated materials which have very little yellowing in comparison with materials treated according to the prior art, and have a whiteness index which is very close to that of the untreated material.

## Claims

1. A method of treating fibrous materials which comprises the application to the fibrous materials of a composition comprising an amine containing organosilicon compound, characterised in that the sole amine containing organosilicon compound in the composition is the reaction product of an organopolysiloxane having at least one unit of the general formula and at least one unit of the general formula with one or more monoepoxides wherein X denotes a monovalent hydrocarbon group having up to 8 carbon atoms, R denotes a divalent alkylene group, R'denotes a hydrogen atom or a group of the formula RZ wherein Z is NHX, NH₂, NHRNH₂ or NHRNHX, a has a value of 1 or 2 and has a value of 2 or 3.

2. A method according to Claim 1 characterised in that the organopolysiloxane is a substantially linear polydiorganosiloxane wherein at least 80% of all X groups are methyl groups.

3. A method according to either Claim 1 or Claim 2 characterised in that the organopolysiloxane comprises from 100 to 500 siloxane units.

4. A method according to any one of the preceding claims characterised in that from 1 to 10 mole% of all siloxane units of the organopolysiloxane are units of the formula 03₋aSiXₐRNHR'. 2

5. A method according to any one of the preceding claims characterised in that the monoepoxide has the general formula wherein n has a value of from 0 to 8.

6. A method according to any one of the preceding claims characterised in that the majority of amine groups in the reaction product are tertiary amine groups, there being no more than 10% primary amine groups present in said reaction product.

7. A method according to any one of the preceding claims characterised in that the reaction product does not contain any primary or secondary amine groups.

8. A method according to any one of the preceding claims characterised in that the composition is in the form of an emulsion.

9. A method according to any one of the preceding claims characterised in that the composition comprises no other amine containing compounds than the reaction product.

10. Textiles incorporating fibres characterised in that the fibres have been treated by a method according to any one of the preceding claims.

## Patentansprüche

1. Verfahren zur Behandlung von faserförmigen Materialien, umfassend das Aufbringen einer Zusammensetzung umfassend eine Amingruppen enthaltende Organosiliciumverbindung auf das faserförmige Material, dadurch gekennzeichnet, daß die einzige Amingruppen enthaltende Organosiliciumverbindung in der Zusammensetzung das Reaktionsprodukt eines Organopolysiloxans mit mindestens einer Einheit der allgemeinen Formel und mindestens einer Einheit der allgemeinen Formel 2 2 mit einem oder mehreren Monoepoxiden ist, wobei X eine monovalente Kohlenwasserstoffgruppe mit bis zu 8 Kohlenstoffatomen bedeutet, R eine divalente Alkylengruppe bedeutet, R' ein Wasserstoffatom oder eine Gruppe der Formel RZ bezeichnet, worin Z NHX, NH₂, NHRNH₂ oder NHRNHX ist, a einen Wert von 1 oder 2 hat und b einen Wert von 2 oder 3 hat.

2. Verfahren nach Anspruch 1, dadurch gekennzeichnet, daß das Organopolysiloxan ein im wesentlichen lineares Polydiorganosiloxan ist, worin mindestens 80% aller Gruppen X Methylgruppen sind.

3. Verfahren nach Anspruch 1 oder Anspruch 2, dadurch gekennzeichnet, daß das Organopolysiloxan 100 bis 500 Siloxaneinheiten umfaßt.

4. Verfahren nach einem der vorhergehenden Ansprüche, dadurch gekennzeichnet, daß 1 bis 10 Mol-% aller Siloxaneinheiten des Organopolysiloxans Einheiten der Formel 0³₋asiX,-R-NH-R' sind.

5. Verfahren nach einem der vorhergehenden Ansprüche, dadurch gekennzeichnet, daß das Monoepoxid die allgemeine Formel hat, worin n einen Wert von 0 bis 8 hat.

6. Verfahren nach einem der vorhergehenden Ansprüche, dadurch gekennzeichnet, daß die meisten Amingruppen in dem Reaktionsprodukt tertiäre Amingruppen sind, wobei nicht mehr als 10% primäre Amingruppen in dem Reaktionsprodukt vorhanden sind.

7. Verfahren nach einem der vorhergehenden Ansprüche, dadurch gekennzeichnet, daß das Reaktionsprodukt keine primären oder sekundären Amingruppen enthält.

8. Verfahren nach einem der vorhergehenden Ansprüche, dadurch gekennzeichnet, daß die Zusammensetzung in Form einer Emulsion vorliegt.

9. Verfahren nach einem der vorhergehenden Ansprüche, dadurch gekennzeichnet, daß die Zusammensetzung keine anderen Amingruppen enthaltenden Verbindungen als das Reaktionsprodukt enthält.

10. Textilien beinhaltend Fasern, dadurch gekennzeichnet, daß die Fasern mit einem Verfahren gemäß einem der vorhergehenden Ansprüche behandelt wurden.

## Revendications

1. Un procédé de traitement de matières fibreuses qui comprend l'application aux matières fibreuses d'une composition comprenant un composé organosilicié aminé, caractérisé en ce que le seul composé organosilicié aminé contenu dans la composition est le produit réactionnel d'un organopolysiloxane ayant au moins un motif de la formule générale et au moins un motif de la formule générale avec un ou plusieurs monoépoxydes, où X représente un groupe hydrocarboné monovalent ayant jusqu'à 8 atomes de carbone, R représente un groupe alkylène divalent, R' représente un atome d'hydrogène ou un groupe de la formule RZ où Z est NHX, NH₂, NHRNH₂ ou NHRNHX, la valeur de a est 1 ou 2 et la valeur de b est 2 ou 3.

2. Un procédé selon la revendication 1, caractérisé en ce que l'organopolysiloxane est un polydiorganosiloxane sensiblement linéaire dans lequel au moins 80 % de tous les groupes X sont des groupes méthyle.

3. Un procédé selon la revendication 1 ou la revendication 2, caractérisé en ce que l'organopolysiloxane comprend 100 à 500 motifs siloxanes.

4. Un procédé selon l'une quelconque des revendications précédentes, caractérisé en ce que 1 à 10 mol % de tous les motifs siloxanes de l'organopolysiloxane sont des motifs de la formule 03₋aSiXₐRNHR'. 2

5. Un procédé selon l'une quelconque des revendications précédentes, caractérisé en ce que le monoépoxy- de répond à la formule générale où la valeur de n est de 0 à 8.

6. Un procédé selon l'une quelconque des revendications précédentes, caractérisé en ce que la majorité des groupes amino présents dans le produit réactionnel sont des groupes amino tertiaires, le produit réactionnel ne contenant pas plus de 10 % de groupes amino primaires.

7. Un procédé selon l'une quelconque des revendications précédentes, caractérisé en ce que le produit réactionnel ne contient aucun groupe amino primaire ou secondaire.

8. Un procédé selon l'une quelconque des revendications précédentes, caractérisé en ce que la composition est sous la forme d'une émulsion.

9. Un procédé selon l'une quelconque des revendications précédentes, caractérisé en ce que la composition ne comprend pas d'autres composés aminés que le produit réactionnel.

10. Textiles comprenant des fibres, caractérisés en ce que les fibres ont été traitées par un procédé selon l'une quelconque des revendications précédentes.
